# EUROPEAN PATENT APPLICATION

(11) **EP 1 619 235 A1**
(43) Date of publication of application: **25.01.2006**
(21) Application number: 05254411.1
(22) Date of filing: 14.07.2005
(51) Int. Cl.: C10M 169/04, C10M 145/14, B60K 17/00

(54) **Polyalkylmethacrylate polymer as filtration improver**

(30) Priority: 21.07.2004 GB 0416319
(71) Applicant: Afton Chemical Limited, Bracknell, Berkshire RG12 2UW (GB)
(72) Inventor: Clague, Nicholas Paul, Bracknell, Berkshire RG12 9YB (GB)
(74) Representative: Cresswell, Thomas Anthony

(57) **Abstract**

Use of a C₁₂₋₂₀ polyalkyl methacrylate polymer as a lubricating oil additive such that the C₁₂₋₂₀ polyalkyl methacrylate polymer accounts for 0.1 to 0.3 % by weight of the finished lubricating oil, which use comprises the addition of said C₁₂₋₂₀ polyalkyl methacrylate polymer to a lubricating oil based on mineral oil to improve the filtration of said lubricating oil based on mineral oil.

## Description

The invention relates to the use of a composition as a lubricating oil additive to improve the filtration of oils based on mineral oils.

Wear is the loss of metal between surfaces moving relative to each other. Wear occurs in all equipment that has moving parts and if it continues, can lead to equipment malfunction. Lubricant compositions are commonly applied to the metal surfaces of mechanical equipment that features the movement and contact of metal surfaces, for example, in the rolling-sliding contacts of hard steel surfaces. This reduces wear and other damage such as micro-pitting (sometimes called "frosting", "greystaining" or "peeling") which can occur in rolling element bearings and most often on gear teeth, which can lead to significant practical problems such as scuffing, and even to tooth fractures of gears.

The primary function of a gear lubricant is to protect both gears and axles against micro-pitting, fatigue, scoring and wear and to provide a high degree of reliability and durability in the service life of gear equipment. In the automotive industry gear lubricants may also contribute to improving the fuel economy of vehicles by improving the axle efficiency.

A large number of dewaxing aids are commercially available for use as oil additives. One series of such aids is sold under the name Viscoplex®. Included in this series of dewaxing aids are Viscoplex® 9-144, Viscoplex® 9-300, Viscoplex® 9-303 and Viscoplex® 9-305, each of which is described as a viscous concentrate of polyalkyl methacrylate in a solvent-refined neutral oil. Each of these is for use in dewaxing oils as part of the refining process for producing mineral oil base-stock, and each is also said to have the properties of improving filtration speed and oil yield in the dewaxing process, improving the low temperature properties of the resulting base stock, improving the yield of dewaxed oil, increasing oil through-put, reducing the oil content in wax produced and reducing the risk of slack-wax formation on filters. Viscoplex 9-305® is used largely for the purpose of modifying the flow of crude oil through pipelines.

US 6,495,495 B1 discloses the use of a blend comprising from about 30 to about 70 % (preferably 50 %) of an alkyl ester polymer (preferably an ethylene-vinyl acetate copolymer) and from about 70 to about 30 % (preferably 50 %) naphthenic oil as a filterability improver.

Oil products based on mineral oil in the transportation industry generally contain levels of dissolved paraffins (waxes), which are soft and flexible. At low temperatures, these paraffins can begin to precipitate which causes an increase in the viscosity of the product, reducing its ability to flow. In certain diesel engines, for example those that feature a filter, this can also lead to blockages.

The present invention is based on the surprising appreciation that certain concentrations of a particular C₁₂₋₂₀ polyalkyl methacrylate polymer, such as may be obtained from RohMax under Viscoplex 9-305®, may be included in a lubricating oil based on mineral oil, such as a gear oil, with the result that a significant improvement in filtration performance is observed when the composition is used as an additive to the lubricating oil based on mineral oil.

Accordingly, the present invention provides for the use of a C₁₂₋₂₀ polyalkyl methacrylate polymer as a lubricating oil additive such that the C₁₂₋₂₀ polyalkyl methacrylate polymer accounts for 0.1 to 0.3 % by weight of the finished lubricating oil, to improve the filtration of the lubricating oil based on mineral oil. The C₁₂₋₂₀ polyalkyl methacrylate polymer may be used in the form of a composition comprising a mineral carrier oil. In a preferred aspect the invention relates to the use of a composition comprising a C₁₂₋₂₀ polyalkyl methacrylate polymer in a mineral carrier oil to improve the filtration of a lubricating oil based on mineral oil. Preferably the composition accounts for 0.2 to 0.5 % by weight of the finished lubricating oil. Typically, the composition comprises 40 to 50 % by weight of the C₁₂₋₂₀ polyalkyl methacrylate polymer and 50 to 60 % by weight of the mineral carrier oil. Preferably, the composition consists of about 45 % by weight of the C₁₂₋₂₀ polyalkyl methacrylate polymer and about 55 % by weight of the mineral carrier oil. The use according to the present invention results in a finished lubricating oil that exhibits a significant improvement in filtration performance.

The present invention also provides for a finished lubricating oil that results from use according to the invention as defined above, a composition for use according to the invention as defined above, a method of lubricating a metal surface comprising applying said finished lubricating oil to the metal surface, a gear or axle that has been lubricated as defined in said method, and an additive pack comprising a composition for use according to the invention as defined above.

In a preferred embodiment of the use according to the present invention the composition comprising the C₁₂₋₂₀ polyalkyl methacrylate polymer has a viscosity of 500 to 1000 mm²/s. More preferably, the composition has a viscosity of about 800 mm²/s (ASTM D4052) at 100 °C.

In one preferred embodiment the present invention provides for the use of a C₁₂₋₂₀ polyalkyl methacrylate polymer as defined above wherein the lubricating oil based on mineral oil is a gear oil. Accordingly, the finished lubricating oil that results from use according to the present invention is preferably for use in gear oil formulation applications.

In another preferred embodiment of the present invention, the finished lubricating oil that results from use according to the present invention meets the specification by Scania (STO 1:0). This specification requires that the oil to be tested is filtered through a 5 micron (pore size) cellulose membrane in the CETOP RP 124H test, wherein a minimum result of 90 % is required in stage 2 in order for the specification to be met. CETOP stage 2 gives a measurement of filterability and provides the ratio (expressed as a percentage) of the flow rates through the membrane at the end of and at the beginning of the test. A filtration measurement may also be expressed as a volume, wherein the volume represents the amount of oil filtered over a given period of time. It should be noted that repeatability is not good (especially for particularly low or high viscosity fluids) and therefore for each experiment at least three runs are conducted. Accordingly, the finished lubricating oil that results from use according to the present invention exhibits a mean of at least 3 CETOP stage 2 test values of over 90 %. More preferably, this finished lubricating oil meets the specification by Scania (STO 1:0).

In the present invention the finished lubricating oil that results from the use according to the invention as defined above is for use as a lubricant. Preferably, it is a formulated gear oil lubricant composition, for instance for transmissions such as automobile rear axles and manual and automatic gear boxes. More preferably this gear oil composition is formulated to meet the specification by Scania (STO 1:0) for the rear axle and manual gear box of diesel engined automobiles.

Typical treat rates at which the C₁₂₋₂₀ polyalkyl methacrylate polymer is used include 0.09 % and above such as 0.14 and 0.18 %. In another preferred embodiment of the use according to the present invention, the C₁₂₋₂₀ polyalkyl methacrylate polymer is used at a treat rate such that it accounts for 0.1 to 0.2 % by weight of the finished lubricating oil. Typically, the C₁₂₋₂₀ polyalkyl methacrylate polymer accounts for 0.1, 0.15 or 0.2 % by weight of the finished lubricating oil. More preferably, the C₁₂₋₂₀ polyalkyl methacrylate polymer accounts for 0.15 or 0.2 % by weight of the finished lubricating oil. The optimum treat rate will vary according to the nature of the mineral base oil and may be determined on a case-by-case basis by use of the CETOP stage 2 test.

In another preferred embodiment the present invention provides for the use of a composition of the invention as defined above wherein the composition is used at a treat rate such that it accounts for 0.2 to 0.4 % by weight of the finished lubricating oil. Typically, the composition accounts for 0.2, 0.3 or 0.4 % by weight of the finished lubricating oil. More preferably, the composition accounts for 0.3 or 0.4 % by weight of the finished lubricating oil. The optimum treat rate will vary according to the nature of the mineral base oil and may be determined on a case-by-case basis by use of the CETOP stage 2 test.

In another preferred embodiment of the use according to the present invention the lubricating oil based on mineral oil is for automotive or industrial applications. In another preferred embodiment of the use according to the present invention, the lubricating oil based on mineral oil has a viscosity of 80W-90 or 85W-140. In another preferred embodiment of the use according to the present invention the lubricating oil based on mineral oil is a part synthetic base stock. In another preferred embodiment of the use according to the present invention the lubricating oil based on mineral oil comprises brightstock. Preferably, the lubricating oil based on mineral oil is Kuwait Petroleum Company, Respol YPF, Total, Esso or SAFOR base stock. More preferably, the lubricating oil based on mineral oil is a wax-containing base stock.

In another preferred embodiment of the use according to the present invention the lubricating oil based on mineral oil and/or the finished oil comprises a further additive, which further additive is added to the lubricating oil based on mineral oil or the finished lubricating oil prior to, simultaneously with or subsequently to the C₁₂₋₂₀ polyalkyl methacrylate polymer.

The present invention also provides for a method of lubricating a metal surface comprising applying to the metal surface a finished lubricating oil of the present invention as defined above. Preferably the metal surface is that of a gear or axle. More preferably the metal surface is that of a gear or rear axle. Typically, the method comprises adding to and operating a transmission or axle a finished lubricating oil of the invention as defined above.

The present invention also provides for an additive pack comprising a C₁₂₋₂₀ polyalkyl methacrylate polymer for use according to the invention as defined above. The additive pack is added to a lubricating oil based on mineral oil such that the C₁₂₋₂₀ polyalkyl methacrylate polymer accounts for 0.1 to 0.3 % by weight of the finished lubricating oil. Preferably, the additive pack is added to the lubricating oil based on mineral oil such that the contents of the additive pack account for up to 15 % by weight of the finished lubricating oil. Typically, the additive pack is added to the lubricating oil based on mineral oil such that the contents of the additive pack account for 4 to 10 % by weight of the finished lubricating oil. Such an additive pack may comprise any oil additive known to a person skilled in the art that does not interfere with the performance of the C₁₂₋₂₀ polyalkyl methacrylate polymer when used accordance with the present invention as defined above. Examples of appropriate additives are illustrated in the Examples below, wherein a composition of the invention as defined above for use according to the present invention is shown to work in a variety of blends with numerous different additives. Other appropriate additives that may be used in conjunction with the present invention will be evident to the person skilled in the art and include pour point depressants, anti-wear additives, anti-oxidation additives, anti-rust additives, dispersants, boronated dispersants, HiTEC 381 (a fully formulated gear package), viscosity index improvers, detergents and friction modifiers.

The composition for use according to the invention as defined above is preferably in the form of a concentrate. In another preferred embodiment this concentrate is combined with a dispersant. Suitable dispersants will be evident to the person skilled in the art.

The present invention additionally includes machines lubricated by the lubricating oil described above. Although the machine may be any machine for which the inventive lubricating oil would provide satisfactory lubrication, it is envisioned that such machinery would include gas engines, diesel engines, turbine engines, automatic transmissions, manual transmissions, hypoid axles, and gear boxes. Furthermore, the present invention includes vehicles comprising the inventive oil soluble lubricant additive package described above.

Further, the present invention provides a method for lubricating moving parts of a machine comprising the step of: contacting at least one moving part with a lubricant comprising the oil soluble lubricant additive package described above. Although the method may be successfully employed on a wide variety of machines, it is envisioned that such machinery would include: gas engines, diesel engines, turbine engines, automatic transmissions, manual transmissions, hypoid axles, and gear boxes.

It is also useful herein that at least one dispersant used in the oil soluble lubricant additive package described above has a molecular weight of from about 1,000 to about 20,000 amu. In one embodiment the at least one dispersant is a maleic anhydride functionalized polyisobutylene polymer that has been reacted with a polyamine. Also the at least one dispersant can be a product of a Mannich reaction. It is further equally possible that the at least one dispersant is an ethylene-propylene type dispersant.

It is further preferred in one embodiment that the oil soluble lubricant additive package described above additionally comprise at least one component selected from the group consisting of: viscosity index improvers and pour point depressants.

The present invention also includes machines lubricated by the lubricating oil described above. Although the inventive lubricating oil can be used on a wide variety of machines, it is envisioned that the machines especially suited for lubrication include: gas engines, diesel engines, turbine engines, automatic transmissions, manual transmissions, hypoid axles, and gear boxes.

Additionally, the present invention includes vehicles comprising the oil soluble lubricant additive package described above.

A method for lubricating moving parts of a machine is also provided comprising the step of: contacting at least one moving part with a lubricant comprising the oil soluble lubricant additive package described above. Although the method may be employed with a wide variety of machines, it is believed that the method is especially suited for use with: gas engines, diesel engines, turbine engines, automatic transmissions, manual transmissions, hypoid axles, and gear boxes.

The present invention also includes machines lubricated by the lubricating oil described above. Although a wide variety of machines may be lubricated by the present inventive lubricating oil, it is preferred that the machine is selected from the group consisting of: gas engines, diesel engines, turbine engines, automatic transmissions, manual transmissions, hypoid axles, and gear boxes.

It is preferred that the lubricating oil additionally comprises at least one additive selected from the group consisting of: detergents, dispersants, antioxidants, friction modifiers, viscosity index improvers, and pour point depressants.

In accordance with the foregoing summary, the following presents a detailed description of the preferred embodiment of the invention that is currently considered to be the best mode.

The mineral oils useful in this invention can include but are not limited to all common mineral oil base stocks. This would include oils that are naphthenic or paraffinic in chemical structure. Oils that are refined by conventional methodology using acid, alkali, and clay or other agents such as aluminum chloride, or be extracted oils produced, for example, by solvent extraction with solvents such as phenol, sulfur dioxide, furfural, dichlorodiethyl ether, etc. They may be hydrotreated or hydrorefined, dewaxed by chilling or catalytic dewaxing processes, or hydrocracked. The mineral oil may be produced from natural crude sources or be composed of isomerized wax materials or residues of other refining processes. In one embodiment, the oil of lubricating viscosity is a hydrotreated, hydrocracked and/or iso-dewaxed mineral oil having a Viscosity Index (VI) of greater than 80, preferably greater than 90; greater than 90 volume % saturates and less than 0.03 wt. % sulfur.

Group II and Group III basestocks are also particularly suitable for use in the present invention, and are typically prepared from conventional feedstocks using a severe hydrogenation step to reduce the aromatic, sulfur and nitrogen content, followed by dewaxing, hydrofinishing, extraction and/or distillation steps to produce the finished base oil. Group II and III basestocks differ from conventional solvent refined Group I basestocks in that their sulfur, nitrogen and aromatic contents are very low. As a result, these base oils are compositionally very different from conventional solvent refined basestocks. The American Petroleum Institute has categorized these different basestock types as follows: Group I, >0.03 wt. % sulfur, and/or <90 vol% saturates, viscosity index between 80 and 120; Group II, ≤ 0.03 wt. % sulfur, and ≥ 90 vol% saturates, viscosity index between 80 and 120; Group III, ≤ 0.03 wt. % sulfur, and ≥ 90 vol% saturates, viscosity index > 120; Group IV, poly-alpha-olefins. Hydrotreated basestocks and catalytically dewaxed basestocks, because of their low sulfur and aromatics content, generally fall into the Group II and Group III categories.

There is no limitation as to the chemical composition of the various basestocks used in the present invention. For example, the proportions of aromatics, paraffinics, and naphthenics in the various Group I, Group II and Group III oils can vary substantially. The degree of refining and the source of the crude used to produce the oil generally determine this composition. In one embodiment, the base oil comprises a mineral oil having a VI of at least 110.

The lubricating oils may be derived from refined, re-refined oils, or mixtures thereof. Unrefined oils are obtained directly from a natural source or synthetic source (e.g., coal, shale, or tar sands bitumen) without further purification or treatment. Examples of unrefined oils include shale oil obtained directly from a retorting operation, petroleum oil obtained directly from distillation, or an ester oil obtained directly from an esterification process, each of which is then used without further treatment. Refined oils are similar to the unrefined oils except that refined oils have been treated in one or more purification steps to improve one or more properties. Suitable purification techniques include distillation, hydrotreating, dewaxing, solvent extraction, acid or base extraction, filtration, and percolation, all of which are known to those skilled in the art. Re-refined oils are obtained by treating used oils in processes similar to those used to obtain the refined oils. These re-refined oils are also known as reclaimed or reprocessed oils and are often additionally processed by techniques for removal of spent additives and oil breakdown products:

### VISCOSITY INDEX IMPROVERS

Viscosity index improvers impart high and low temperature operability to the lubricating oil and permit it to remain relatively viscous at elevated temperatures and also exhibit acceptable viscosity or fluidity at low temperatures. Viscosity index improvers are generally high molecular weight hydrocarbon polymers including polyesters. The viscosity index improvers may also be derivatized to include other properties or functions, such as the addition of dispersancy properties. These oil soluble viscosity modifying polymers will generally have number average molecular weights of from 10³ to 10⁶, preferably 10⁴ to 10⁶, as determined by gel permeation chromatography or osmometry.

The viscosity index improvers useful herein can include polymethacrylate-based ones, olefin copolymer-based ones, (e.g., isobutylene-based and ethylene-propylene copolymer based ones), polyalkyl styrene-based ones, hydrogenated styrene-butadiene copolymer-based ones, and styrene-maleic anhydride ester copolymer-based ones.

Representative examples of suitable viscosity index improvers are found in U.S. Pat. Nos. 5,075,383; 5,102,566; 5,139,688; 5,238,588; and 6,107,257. The above references are incorporated herein by reference.

### POUR POINT DEPRESSANTS

Pour point depressants are used to improve low temperature properties of oilbased compositions. See, for example, page 8 of "Lubricant Additives" by C.V. Smalheer and R. Kennedy Smith (Lezius Hiles Co. publishers, Cleveland, Ohio, 1967). Examples of useful pour point depressants are polymethacrylates; polyacrylates; polyacrylamides; condensation products of haloparaffin waxes and aromatic compounds; vinyl carboxylate polymers; and ter-polymers of dialkylfumarates, vinyl esters of fatty acids and alkyl vinyl ethers. Pour point depressants are described in U.S. Patent Nos. 2,387,501; 2,015,748; 2,655,479; 1,815,022; 2,191,498; 2,666,746; 2,721,877; 2,721,878; and 3,250,715, which are herein incorporated by reference for their relevant disclosures.

### DISPERSANTS

Dispersants used in the present invention may be ash-producing or ashless. Suitable dispersants for use herein can typically comprise amine, alcohol, amide, or ester polar moieties attached to the polymer backbone via a bridging group. The dispersant may be, for example, selected from oil-soluble salts, esters, amino-esters, amides, imides, and oxazolines of long chain hydrocarbon substituted mono- and dicarboxylic acids or their anhydrides; thiocarboxylate derivatives of chain hydrocarbons; long chain aliphatic hydrocarbons having a polyamine attached directly thereto; and Mannich condensation products formed by condensing a long chain substituted phenol with formaldehyde and polyalkylene polyamine, and Koch reaction products. The long chain aliphatic hydrocarbons can be polymers such as polyalkylenes, including, for example, polyisobutylene, polyethylene, polypropylene, and copolymers thereof and/or copolymers with other alpha-olefins. Typical PIB molecular weights useful herein can range from about 950 to 6000.

Representative examples of dispersants suitable for use in the present invention are found in U.S. Patent Nos. 5,075,383; 5,139,688; 5,238,588; and 6,107,257. Additional representative examples are found in U.S. Patent Application Publication No. 2001/0036906A1. The disclosures of the afore-mentioned references are incorporated herein by reference.

### DETERGENTS

A detergent is an additive that reduces the formation of piston deposits, for example high-temperature varnish and lacquer deposits, in engines. Detergents typically possess acid-neutralizing properties and are capable of keeping finely divided solids in suspension. Metal detergents are used preferably for improving the acid-neutralizing properties, high-temperature detergency, and anti-wear properties of the resulting lubricating oil composition.

Detergents used herein may be any detergent used in lubricating oil formulations, and may be of the ash-producing or ashless variety. Detergents suitable for use in the present invention include all of the detergents customarily used in lubricating oils, including metal detergents. Specific examples of metal detergents are those selected from alkali metal or alkaline earth metal sulfonates, alkali metal or alkaline earth metal phenates, and alkali metal or alkaline earth metal salicylates. In an embodiment, the lubricating oil formulation is essentially free of sulfurized phenate detergent.

Representative examples of suitable detergents useful in the present invention are found in U.S. Pat. Nos. 6,008,166. Additional representative examples of suitable detergents are found in U.S. Patent Application Nos. 2002/0142922A1, 2002/0004069A1, and 2002/0147115A1. The disclosures of the afore-mentioned references are incorporated by reference herein.

### ANTIOXIDANTS

Useful antioxidant materials include oil soluble phenolic compounds, oil soluble sulfurized organic compounds, oil soluble amine antioxidants, oil soluble organo borates, oil soluble organo phosphites, oil soluble organo phosphates, oil soluble organo dithiophosphates and mixtures thereof. Such antioxidants can be metal free (that is, free of metals which are capable of generating sulfated ash), and therefore are most preferably ashless (having a sulfated ash value not greater than 1 wt. % SASH, as determined by ASTM D874).

Representative examples of suitable antioxidants useful in the present invention are found in U.S. Patent No. 5,102,566. Additional representative examples of suitable antioxidants useful in the present invention are found in U.S. Patent Application Publication No. 2001/0012821A1. The disclosures of the afore-mentioned references are incorporated by reference herein.

### FRICTION MODIFIERS

Friction modifiers serve to impart the proper friction characteristics to lubricating oil compositions.

Friction modifiers include such compounds as aliphatic amines or ethoxylated aliphatic amines, aliphatic fatty acid amines, aliphatic carboxylic acids, aliphatic carboxylic esters of polyols such as glycerol esters of fatty acid as exemplified by glycerol phenate, aliphatic carboxylic ester-amides, aliphatic phosphonates, aliphatic phosphates, aliphatic thiophosphonates, aliphatic thiophosphates, etc., wherein the aliphatic group usually contains above about eight carbon atoms so as to render the compound suitably oil soluble. Also suitable are aliphatic substituted succinimides formed by reacting one or more aliphatic succinic acids or anhydrides with ammonia. Additionally suited for use in the present invention are friction modifiers containing molybdenum.

Representative examples of molybdenum-containing friction modifiers include those found in U.S. Patent Nos. 5,650,381; RE37,363E; 5,628,802; 4,889,647; 5,412,130; 4,786,423; 4,812,246; 5,137,647; 5,364,545; 5,840,672; 5,925,600; 5,962,377; 5,994,277; 6,017,858; 6,150,309; 6,174,842; 6,187,723; 6,268,316; European Patent Nos. EP 222 143 B1; EP 281 992 B1; EP 719 314 B1; EP 719 315 B1; EP 874 040 A1; EP 892 037 A1; EP 931 827 A1; EP 1 041 134 A1; EP 1 041 135 A1; EP 1 087 008 A1; EP 1 088 882 A1; EP; Japanese Patent No. JP 11035961; and International Publication Nos. WO 95/07965; WO 00/08120; WO 00/71649.

Representative examples of suitable friction modifiers are found in U.S. Pat. Nos. 3,933,659; 4,105,571; 3,779,928; 3,778,375; 3,852,205; 3,879,306; 3,932,290; 3,932,290; 4,028,258; 4,344,853; 5,102,566; 6,103,674; 6,174,842; 6,500,786; 6,500,786; and 6,509,303. Additional representative examples of suitable friction modifiers are found in U.S. Patent Application Publication No. 2002/0137636 A1. The disclosures of the above references are incorporated herein by reference.

### EXAMPLES

The invention is illustrated by the following examples.

Lubricant compositions were prepared by blending the components present as indicated below. The results are shown in Tables 1 to 3 below. Filtration measurements are expressed either as a percentage or as a volume, as described above. A new 5 micron cellulose filter membrane was used for each test.

The results exemplified in the Tables 1 to 3 illustrate the significant improvement in filtration performance exhibited by blends that comprise a C₁₂₋₂₀ polyalkyl methacrylate polymer at the appropriate concentrations. In conjunction with Table 5 it is of note that the Shell base stocks meet the specification by Scania without the addition of a C₁₂₋₂₀ polyalkyl methacrylate polymer at the appropriate concentrations. This is because the Shell base stock is filtered to remove the wax during the manufacturing process. In any case, the addition to this base stock of a C₁₂₋₂₀ polyalkyl methacrylate polymer at the appropriate concentrations did not result in any detrimental effect to the filterability of the finished oil blend and the finished lubricating oil resulting from the addition to the Shell base stock of a C₁₂₋₂₀ polyalkyl methacrylate polymer at the appropriate concentrations was shown to meet the specification by Scania (STO 1:0).

The properties of certain components (as used in the above experiments and in the industry in general) are as follows:

## Claims

1. Use of a C₁₂₋₂₀ polyalkyl methacrylate polymer as a lubricating oil additive such that the C₁₂₋₂₀ polyalkyl methacrylate polymer accounts for 0.1 to 0.3 % by weight of the finished lubricating oil, which use comprises the addition of said C₁₂₋₂₀ polyalkyl methacrylate polymer to a lubricating oil based on mineral oil to improve the filtration of said lubricating oil based on mineral oil.

2. Use according to claim 1 wherein the lubricating oil based on mineral oil is a gear oil.

3. Use according to claim 1 or 2 wherein the mean CETOP filtration stage 2 test value of the finished lubricating oil (the oil resulting from said use) is over 90 %.

4. Use according to claim 3 wherein the finished lubricating oil (the oil resulting from said use) meets the specification by Scania (STO 1:0).

5. Use according to any one of claims 1 to 4 wherein the C₁₂₋₂₀ polyalkyl methacrylate polymer accounts for 0.1 or 0.2 % by weight of the finished lubricating oil.

6. Use according to any one of the preceding claims of a composition comprising the C₁₂₋₂₀ polyalkyl methacrylate polymer.

7. Use according to claim 6 wherein the composition comprises about 45 % by weight of the C₁₂₋₂₀ polyalkyl methacrylate polymer and about 55 % by weight of a mineral carrier oil.

8. Use according to claim 7 wherein the composition has a viscosity of 800 mm²/s (ASTM D4052) at 100 °C.

9. Use according to any one of the preceding claims wherein the lubricating oil based on mineral oil has a viscosity of 80W-90 or 85W-140.

10. Use according to any one of claims 1 to 8 wherein the lubricating oil based on mineral oil is for automotive or industrial applications.

11. Use according to any one of the preceding claims wherein the lubricating oil based on mineral oil is a part synthetic base stock.

12. Use according to any one of the preceding claims wherein the lubricating oil based on mineral oil comprises brightstock.

13. Use according to any one of the preceding claims wherein the lubricating oil based on mineral oil is Kuwait Petroleum Company, Repsol YPF, Total, Esso or SAFOR base stock.

14. Use according to any one of the preceding claims wherein the lubricating oil based on mineral oil and/or the finished lubricating oil comprises a further additive, which further additive is added to the lubricating oil based on mineral oil or the finished lubricating oil prior to, simultaneously with or subsequently to the composition comprising a C₁₂₋₂₀ polyalkyl methacrylate polymer in a mineral carrier oil.

15. Use according to any one of the preceding claims wherein the lubricating oil based on mineral oil is a formulated gear lubricant composition.

16. A finished lubricating oil resulting from a use as defined in any one of claims 1 to 15.

17. A method of lubricating the metal surface of a gear or axle comprising applying to the metal surface a finished lubricating oil as defined in claim 16.

18. A method according to claim 17 wherein the method comprises adding a finished lubricating oil as defined in claim 16 to a transmission or axle and operating the transmission or axle.

19. A gear or axle which has been lubricated in a method according to claim 17 or 18.

20. A composition comprising a C₁₂₋₂₀ polyalkyl methacrylate polymer in a mineral carrier oil for use as defined in any one of claims 1 to 15.

21. A gear additive package comprising a composition as defined in claim 20.
